

## UNITED STATES PATENT OFFICE

2,030,904

PHOTOGRAPHIC FILM OF THE MONOPACK  
TYPE ADAPTED FOR COLOR PHOTOGRAPHYHans von Fraunhofer, New York, N. Y., assignor  
to Omnidrome Corporation, New York, N. Y.,  
a corporation of New YorkNo Drawing. Application August 3, 1934.  
Serial No. 738,299

## 11 Claims. (Cl. 95—2)

This invention relates to improvements in photographic films of the mono-pack type adapted for color photography, being particularly directed to sensitized multi-strata films and methods of producing the same.

Up to the present time, considerable difficulty has been encountered in the production of films for color photography, due to the following factors: bi-packs and tri-packs, the separate sections of which are sensitized for different colors, have the mechanical difficulty presented by the necessity for taking two or three exposures simultaneously, plus the inherent difficulty involved in attempting to align different images and color values of the different supports for transposition on a single finished print.

Further, in passing light through one or more carriers in preparation of the final print, there is such a loss due to diffusion, that a clear, balanced and incorporated image and the full color and line values of the subject being photographed are difficult of production; in mono-packs involving emulsions on one or both sides of a carrier considerable discussion has been disclosed in the literature as indicated in "The History of Three-Color Photography" by Wall, and the patents to Troland, Mannes and Godowsky, Kelley, Ives, and others; in, all of such disclosures, various layers or strata to form the mono-pack are superimposed one on top of the other with respect to the carrier, or disposed on opposite sides thereof, and alternate methods are used for producing the sensitized film, as, for example (a) each layer is sensitized for its color value after it has been disposed on its carrier; (b) an emulsion is sensitized for color and then spread upon the carrier on opposite sides thereof or one on top of the other, or (c) a layer of emulsion on a carrier is subjected successively to sensitizers for warmer and colder colors or vice versa, with the result that two layers are formed; in the first of the mono-pack methods difficulty is involved in the intermixture in a plurality of layers or the incomplete distribution in respective layers of the color sensitizing dyes. In the last of such mono-pack methods, there is indicated an ever-present problem in the nature of improper, incomplete and unbalanced diffusion of the sensitizing dyes into the emulsion on the carrier, with the result that the necessary strata formation for images of respective color values approximating the natural, has not to date been produced.

Broadly, it is an object of this invention to provide for a novel form of multi-strata mono-pack film and a simple and efficient method of pro-

ducing the same, involving the application of a sensitizing solution containing sensitizing and filter dyes of color value capable of diffusing into the emulsion in a single step operation to provide the sensitized multi-strata formation necessary to produce images in natural color.

Still further, it is an object of this invention to provide a method of applying a series of sensitizers in a single solution to an emulsion, such sensitizers incorporating dyes in solution, respective particles of which are of different size, whereby the sensitizing solution, that is, the respective sensitizing and filter dyes thereof, are diffused into the emulsion to produce a plurality of strata, each sensitized for a different color value, the components of the sensitizing solution being such for the respective color values as to provide a different rate of diffusion of the dyes imparting the particular color values to the silver salts in the emulsion and color absorption within the emulsion within only certain defined depths or strata; the sensitizing solution being preferably so constituted as to provide for red sensitization at the uppermost or emergent strata, green sensitization for the middle or intermediate strata and blue sensitization for the lowermost or entrance strata. Although the order and arrangement of strata may be reversed by difference in method of application of the sensitizing solution to the emulsion or by difference in particle size and constitution of the respective dyes in such solution.

Specifically, it is an object of this invention to apply to an emulsion a solution comprising a mixture of sensitizing dyes and filter dyes of such composition and so constituted to particle size as to yield upon treatment of a common single layered photographic film, a three-layered stratification of the emulsion of such film, each stratum being so constituted with respect to the silver salt-dye reaction product formed in the stratum as to permit only the reaction, from the standpoint of subtractive analysis, of the silver salt-dye reaction product, with the light of a specific color in each such specific stratum, so that upon treatment of a single layer film with such sensitizing solution, the layer is acted upon to form three strata, each of which is effectively sensitized to analysis for the production of images approximating the natural coloration according to the demands of three color photography.

In general, therefore, this invention contemplates the treatment of a mono-pack film by incorporating in the emulsion thereof in a single operation, dyes for both color sensitization and

filtering, the respective dye particles being of such a nature and so constituted as to be diffused at different rates and proportions into the film emulsion, to produce a multi-layer stratification, 5 in the particular instance, a three-layer stratification of the film emulsion, the silver salt in the respective strata and the strata being sensitized and affected as to provide acceptance by analysis of the primary color components of light 10 so as to produce upon exposure of the film, images incorporating the respective primary colors, in the different strata, and their derivatives, substantially reproducing natural coloration with full clarity and depth.

15 It is to be understood that three-layer stratification and color sensitization thereof, as herein practiced, to produce three-color photography, involves a process of incorporating color dyes in the form of color sensitizers to produce sensitization 20 respectively for the warm colors incorporating red and yellow, but preponderantly red, and colder colors incorporating green and blue, but preponderantly green, plus color filtering media in the form of dyes to respectively control the 25 passage of color components of light up to, within, or beyond respective strata, the respective color sensitized and affected strata thereby providing for the production of images reproducing natural coloration directly and in conjunction 30 with subtractive analysis.

According to my process, I apply to the emulsion of the ordinary black and white monochromatic film a sensitizing solution which may, for the purpose of this disclosure, be considered a 35 colloidal suspension in the form of dye particles in different sizes to provide stratification, and which incorporates in a dispersion medium of alcohol and water color sensitizing and filtering dyes of the following nature and in the following 40 proportion:

For the warmer colors pinacyanol or cyanine, relatively large particles in alcohol;

For the cold colors, pinachrom and Erythrosin in aqueous solution, and Orthochrom T in alcoholic solution, the particles being relatively of 45 small size;

For color filtering, Rose Bengal medium size particles and Rapid Filter Yellow of fine particles, both in aqueous solution.

50 I prefer to use the above specified color sensitizing and filtering dyes in the following quantities, with respect to the dispersing medium: I dissolve 1 g. of Pinorthol 1, which comprises essentially of a mixture of Pinachrom and Erythrosin and a slight amount of Rapid Filter Yellow, 1 g. of Rapid Filter Yellow and .4 g. of rose bengal, in order, in 150 c. c. of water; I then add to the above solution 25 c. c. of 1/1000 alcohol solution of Pinacyanol and 25 c. c. of 1/1000 alcohol solution of Orthochrom T, with stirring, after which I add 200 c. c. of alcohol, and then add water until the solution makes up to 500 c. c., with stirring.

In operation, I sensitize the film by spraying or coating the emulsion, which emulsion may be 65 carried on glass, paper, or celluloid, as applied for different kinds of photography, or the sensitizing solution is sprayed or coated onto a carrier, in the nature of glass, water-proof paper, or celluloid, and a layer of emulsion then deposited thereon; in either case of which the sensitizing solution, that is, the respective constituents thereof, penetrate by diffusion, at rates dependent upon the particle size thereof, into the emulsion, to form three clearly defined strata, in the first of 70 which, the product of the silver salt and the par-

ticles of the sensitizing solution reacting therewith provides for acceptance of the warmer colors, to wit: red and its derivatives; in the next adjacent of which strata, the product of the silver salt and the particles of the sensitization solution reacting therewith provides for the acceptance of the colder color to wit: green and its derivatives, and in the third stratum of which the product of the silver salt and the particles of the sensitizing solution reacting therewith provide 10 for the acceptance of the colder blue color and its derivatives.

To more clearly define the result with respect to the constitution of the three-strata formation of the emulsion after sensitization, it should be 15 noted that the first stratum contains a preponderance of the slowly diffusing Pinacyanol particles, a much smaller amount of the relatively larger and faster diffusing Pinachrom, erythrosin, Orthochrom T, and rose bengal particles, and a 20 very small amount of the fine and swiftly diffusing Rapid Filter Yellow particles, and in such layer the silver salt is essentially and for all practical purposes completely sensitized for only the color red and its derivatives.

25 The next adjacent stratum contains a preponderance of the relatively small erythrosin, Pinachrom and Orthochrom T green sensitizing particles, for reaction with the silver salt in such stratum, together with rose bengal and Rapid 30 Filter Yellow particles which have become diffused throughout the stratum; the Pinacyanol particles being large and slow diffusing do not penetrate into such layer to any effected degree, thus providing a clearly defined stratum sensitized to record green color values only.

35 The next adjacent or third stratum contains a preponderance of Rapid Filter Yellow comprising the fastest moving of all particles, and in such layer the silver salt, being normally predominantly 40 sensitive to blue, becomes effective only to accept the blue component of light.

It is to be understood that the action or effect of rose bengal and Rapid Filter Yellow, the filter dyes, is not considered with relation to 45 the color sensitization of the silver salts in the respective layers and the formation of color images by the reaction product of the sensitizing dyes in the respective strata with such salts, but their action in the respective strata is directed 50 in the subtractive analysis of light upon exposure of the sensitized film to a control for limiting the passage of blue and green components of light beyond the stratum in which such colors are accepted; as, for example, the blue component 55 of light being accepted in the furthermost stratum, by virtue of the presence in such stratum of the silver salt which normally is predominantly sensitive to blue, and which is unaffected by the color sensitizing solution, the Rapid 60 Filter Yellow being minus blue in its characteristics or properties, prevents the passage of blue components into the middle of the green stratum, and the uppermost or red stratum; rose bengal being minus green in its characteristics or properties 65 limits the passage of green component to the intermediate or green sensitized stratum, and prevents the passage of the green light component into the uppermost or red sensitized stratum.

70 Although two methods of sensitizing of the emulsion have been specified, I prefer, from the standpoint of practicability, at the present time, to sensitize by spraying or coating the emulsion already carried on glass, paper or celluloid, al- 75

though the second method described has advantages, particularly in color photography involving a paper film, since it is concededly advantageous to have a blue sensitivity in the entrant stratum, and red sensitivity in the emergent stratum.

Further, I have found it advantageous in the event of the two methods above described for sensitization as applied to pre-wet the emulsion, and for such purpose, I apply a borax solution, the function and application of which is more clearly defined in a co-pending application filed by Joseph S. Friedman August 3rd, 1934, Serial No. 738,214, and assigned to the Omnidochrome Corporation, the assignee of this application. By the use of such reagent for pre-wetting the emulsion, I am enabled to provide an emulsion whose silver salt content is constant, but whose depth is increased several times by the swelling of the 20 gelatine dispersion medium carrying the silver salt in the emulsion, to provide for more thorough and complete diffusion of the respective color sensitizing and filter dyes to the necessary depth.

It is to be understood that by the expression "sensitizing solution" is meant a solution in the nature of a colloidal suspension, incorporating a dispersion medium carrying dyes of relatively different particle size, some of such dyes being capable of sensitizing silver salts in the emulsion of film by chemical reaction for different color values, and others being adapted, upon dispersion within the film emulsion, to serve as color filter media; the sensitizing solution being so constituted upon application to emulsion as to provide diffusion of the dye particles therein, into the emulsion, to form a plurality of contiguous strata in the emulsion, in each of which the silver salt is acted upon or affected so as to provide, upon exposure of the film, for the formation of images of its predetermined specific primary color and derivatives, to the exclusion of all others.

Although I have indicated a specific sensitization solution, I do not limit myself to the use of this solution, or all of the ingredients thereof, together in the same proportion, it being within the province of this invention to vary the number and type of dyes, and the particle size thereof, in the dispersion medium, so long as upon application of such sensitizing solution to an emulsion of a mono-pack film, a multi-layer stratification, particularly a three-layer stratification of the type described, is produced in the manner described.

With respect to the dyes herein mentioned, following is the color index of each thereof as recognized and published under the Society of Dyers and Colourists Color Index: Pinacyanol, No. 808, cyanine, No. 806, Orthochrome T, No. 807, erythrosine, No. 772, rose bengal, No. 777, Rapid Filter Yellow, No. 640.

It is obvious that various changes and modifications may be made to the details of component applied and the process involved without departing from the general spirit of the invention as set forth in the appended claims.

I claim:

1. A method of treating a mono-pack film, comprising diffusing into the emulsion of the film a reagent incorporating sensitizing dyes and filter dyes of such particle size and rate of diffusion for such time as to produce in the emulsion a plurality of strata predominantly sensitized respectively to record different color aspects.

2. A method of treating a mono-pack film, comprising diffusing into the emulsion of the film a reagent, incorporating sensitizing dyes and filter dyes of such particle size and rate of diffusion for such time as to produce in the emulsion a plurality of strata predominantly sensitized respectively to record different color aspects, each stratum being affected to exclude substantially the recordation of color aspects other than its own.

3. A method of treating a mono-pack film, comprising diffusing into the emulsion of the film a reagent incorporating sensitizing dyes and filter dyes of such particle size and rate of diffusion for such time as to produce in the emulsion a three-strata formation, each stratum being predominantly sensitized to record different color aspects, each stratum being affected as to exclude substantially the recordation of color aspects other than its own.

4. A method of making a sensitized mono-pack film for use in color photography, comprising subjecting the emulsion thereof to the action at one time of a single reagent, incorporating color sensitizing dyes and filter dyes of such particle size and rate of diffusion for such time as to produce a multi-strata formation in the emulsion the silver salts in each stratum being affected to record predominantly a specific spectral range, and to be unaffected substantially as to the other spectral ranges recorded in the other strata.

5. A method of making a sensitized mono-pack film for use in color photography, comprising subjecting the emulsion thereof to the action at one time of a single solution incorporating color sensitizing dyes and filter dyes of such particle size and rate of diffusion for such time as to produce a three-strata formation in the emulsion, the silver salts in each stratum being affected to record predominantly a specific spectral range and to be unaffected substantially as to the other spectral ranges recorded in the other strata.

6. A method of sensitizing a mono-pack film for use in color photography, which comprises treating the emulsion of such film with a reagent incorporating color sensitizing dyes of such particle size and rate of diffusion for such time as to produce in the emulsion a plurality of strata predominantly sensitized respectively to record different color aspects.

7. A method of sensitizing a mono-pack film for use in color photography, which comprises treating the emulsion of such film with a reagent incorporating color sensitizing dyes of such particle size and rate of diffusion for such time as to produce in the emulsion a plurality of strata predominantly sensitized respectively to record different color aspects, each stratum being affected as to exclude substantially the recordation of color aspects other than its own.

8. A method of sensitizing a mono-pack film for use in color photography, which comprises treating the emulsion of such film with a reagent incorporating color sensitizing dyes and filter dyes of such particle size and rate of diffusion for such time as to produce in the emulsion a multi-strata formation, each stratum being predominantly sensitized to record different color aspects, the top stratum being affected to record only the red aspect, the intermediate stratum being affected to record only the green aspect, and the lower stratum being affected to record only the blue aspect.

9. A method of sensitizing a mono-pack film for use in color photography, which comprises

- treating the emulsion of such film with a reagent incorporating color sensitizing dyes and filter dyes of such particle size and rate of diffusion for such time as to produce in the emulsion a 5 multi-strata formation, each stratum being predominantly sensitized to record different color aspects, the top stratum being affected to record only the red aspect, the intermediate stratum being affected to record only the green aspect, and 10 the lower stratum being affected to record only the blue aspect, each stratum being affected as to exclude the recordation of color aspects other than that to which the silver salts have been sensitized.
- 15 10. A method of making a sensitized monopack film for use in color photography, comprising a silver halide emulsion upon a support, sub-

jecting the emulsion to a reagent containing color sensitizing dyes and filter dyes, the rate of diffusion of said dyes being controlled by the particle size thereof, whereby a single treatment for a predetermined time produces strata predominantly sensitized for different spectral ranges. 5

11. A method of making a sensitized monopack film for use in color photography, comprising a silver halide emulsion upon a support, subjecting the emulsion to a reagent containing color 10 sensitizing dyes and filter dyes, the rate of diffusion of said dyes being controlled by the particle size thereof, whereby a single treatment for a predetermined time produces strata predominantly sensitized for different spectral 15 ranges.

HANS von FRAUNHOFER.